

## UNITED STATES PATENT OFFICE

2,374,388

## TREATING INHERENTLY AGING CHROMIUM-NICKEL STAINLESS STEEL

George V. Smith, Millburn, N. J., assignor to  
United States Steel Corporation of Delaware,  
a corporation of Delaware

No Drawing. Application July 16, 1943,  
Serial No. 495,029

1 Claim. (Cl. 148—21.5)

This invention is a method of treating chromium-nickel stainless steel containing carbon and at least one of the stronger-than-chromium carbide formers, such as titanium, columbium, zirconium, etc., with its components that are ferrite formers proportioned to those that are austenite formers to cause the production of stress-laden ferrite at low temperatures when the steel cools to room temperature from temperatures where it is completely austenitic. Usually 10 the steel contains aluminum.

As disclosed and claimed in the Wyche and Smith application, filed October 8, 1941, Serial No. 414,194, the stress-laden ferrite, of such a steel, is inherently aging to a much higher hardness and strength. By varying the proportion between the ferrite formers and the austenite formers the steel may be made to contain more or less of this aging ferrite, with the balance austenite, but once the steel is made this is, naturally, impossible.

The present invention is a method of treating such steel so as to decrease the amount of aging ferrite while increasing the nonaging austenite, at the time of aging, by heat treatment, as contrasted to varying the composition of the steel.

According to this invention, steel, of the character described, that has been produced in the normal fashion, so as to obtain the maximum amount of stress-laden ferrite its composition permits, is heated to transform at least some of this ferrite to austenite, and is then cooled to temperatures where this austenite, produced from the aging ferrite, transforms back to the ferrite with time, the steel being then held until a selected and determined proportion of the aging ferrite is produced, whereupon the steel is reheated to temperatures preventing further transformation of this austenite, which would otherwise transform to stress-laden ferrite, which temperatures are adequate to age the ferrite that did transform, the steel being held to at least partially age this ferrite, and then being cooled to room temperature. During the last step some, or all, of the austenite, formed from the stress-laden ferrite, may transform to the stress-laden ferrite, but since no aging step is given this portion of the ferrite, it does not acquire the higher strength and hardness as has that portion

that was aged. It follows that, by proper selection of time and temperature, it is possible to selectively age any given proportion of the aging ferrite so as to, selectively, impart different properties to the steel.

Depending on the exact composition of the steel, temperatures of 1100° to 2200° F. will serve to austenitize the stress-laden ferrite, inherently possessed by the steel, the austenite thus produced retransforming to the stress-laden ferrite at temperatures ranging from 200° downwardly to less than room temperature, the transformation requiring time, which is limited in accordance with the amount of the normally available aging ferrite it is desired to age, while temperatures of from 700° to 1100° F. will serve to completely stop this transformation to the ferrite and to age the ferrite that was allowed to transform. As previously explained, when the steel is finally permitted to cool to room temperature, it may develop all of its stress-laden ferrite, afforded by its composition, but this ferrite will be unaged.

It follows from the foregoing that this invention provides an additional means for adjusting the properties of steel of the type described, other than by adjustment of its chemical composition such as would inherently lead to various amounts of stress-laden or aging ferrite.

I claim:

30 A method of treating chromium-nickel stainless steel containing carbon and at least one of the stronger-than-chromium carbide formers such as titanium, columbium, zirconium, etc., with its components that are ferrite formers proportioned to those that are austenite formers to cause the production of stress-laden ferrite at low temperatures when the steel cools to room temperature from temperatures where it is completely austenitic, said method comprising heating the steel to transform at least some of said ferrite to austenite, cooling the steel to temperatures where said austenite transforms to said ferrite and holding until some but not all of said austenite transforms to said ferrite, reheating to temperatures preventing further transformation of said austenite and which age said ferrite and holding to at least partially age said ferrite, and cooling the steel to room temperature.

GEORGE V. SMITH.